

# UNITED STATES PATENT OFFICE.

BENNO STRAUSS, OF BREDENEY, GERMANY.

## METHOD OF TREATING STEEL ALLOYS WHICH CONTAIN CHROMIUM AND NICKEL.

1,404,908.

Specification of Letters Patent. Patented Jan. 31, 1922.

No Drawing. Original application filed June 25, 1913, Serial No. 775,765. Divided and this application filed June 19, 1914. Serial No. 846,169.

(GRANTED UNDER THE PROVISIONS OF THE ACT OF MARCH 3, 1921, 41 STAT. L., 1313.)

To all whom it may concern:

Be it known that I, BENNO STRAUSS, a citizen of the German Empire, residing at Bredeney, Germany, have invented certain new and useful Improvements in a Method of Treating Steel Alloys which Contain Chromium and Nickel, of which the following is a specification.

This application is a division of my application filed June 25, 1913, Serial No. 775,765.

This invention relates to a method of treating steel alloys, which contain more than 6% chromium, from 20% to  $\frac{1}{2}$ % nickel and not over 1% carbon and which possess a hardness below 350 Brinell scale in the forged state.

According to this invention said steel alloys which when containing from 8% to 25% chromium are either slightly magnetic or else entirely non-magnetic, are heated to a temperature situated between 1100° and 1200° C. and thereupon (quickly or slowly) cooled.

By means of this heating treatment said alloys will obtain a very great toughness and are made easy to work. The slightly mag-

netic alloys will become in addition unmagnetic, when quickly cooled.

I claim:

1. Method of treating steel alloys containing at least 8% chromium, 20% to  $\frac{1}{2}$ % nickel and not over 1% carbon and having a hardness below 350 (Brinell scale) in the forged state, said method consisting in heating the alloys to a temperature from 1100° to 1200° C. and subsequently cooling them, whereby the alloys obtain great toughness. 35

2. Method of treating steel alloys containing 8% to 25% chromium, 20% to  $\frac{1}{2}$ % nickel and not over 1% carbon and having a hardness below 350 (Brinell scale) in the forged state, said method consisting in heating the alloys to a temperature from 1100° to 1200° C. and subsequently cooling them quickly, 40 whereby the alloys are made tough and unmagnetic. 45

In testimony whereof the foregoing specification is signed in the presence of two witnesses.

BENNO STRAUSS. [L. S.]

Witnesses:

ALBERT NUFER,  
FRANCES NUFER.